

## UNITED STATES PATENT OFFICE

LEON WEISBERG, OF PHILADELPHIA, PENNSYLVANIA

## COMPOSITION OF MATTER FOR PUTTY

No Drawing.

Application filed January 14, 1930. Serial No. 420,816.

This invention in general relates to a composition of matter and more particularly to a putty having for its object the provision of an improved composition of the kind indicated with certain desired features which keep the putty in a homogeneous moist condition without the usual seeping of the fluids contained therein to the surface of the solid ingredients employed.

Another object of the invention is to provide a putty which will not cling to the hands of the user which hitherto has entailed much inconvenience both to store-keepers handling putty and to those engaged in actually working and applying it in the different industries.

As is well known, when putty is handled it has a tendency to stick to the fingers of the user entailing considerable time for its removal, and in the case of store-keepers where handling food products necessitating the frequent washing of the hands and the employment of powerful solvents, in order to remove all trace of the oils and pigments which would contaminate food products coming in contact therewith.

In carrying into practice the object of the present invention I employ the following ingredients preferably in the proportions indicated altho I do not confine myself to the precise ratio indicated as this is susceptible of considerable variation. The following composition has been found by me to yield the desirable results indicated above:—

|                                | Pounds |
|--------------------------------|--------|
| Marble dust                    | 25     |
| Whiting                        | 173    |
| Asbestos (ground)              | 6      |
| Special heavy pure linseed oil | 4      |
| Machine oil                    | 1      |
| Paraffin oil                   | 32½    |

The above putty I have found can be kept indefinitely in the usual containers without becoming hard and dry at the bottom and excessively soft on top, which is a defect well known to those handling the conventional putty employed in the various industries at the present time.

The asbestos in the above composition not

only has a tendency to retain the oil homogeneously throughout the composition, but also makes it highly durable and weather resistant where it is employed for outside work.

It will of course be understood that while I have described a putty with a preferred proportioning of ingredients certain slight changes may be made therein without departing from the spirit or sacrificing any of the advantages of the invention, hence I do not confine myself literally thereto, save to the extent indicated within the limits of the appended claim.

Having thus described my invention, what I claim is new and desire to secure by Letters Patent, is:—

A composition of matter of the kind indicated containing the following ingredients as designated,—marble dust 10%, whiting 70%, heavy body pure linseed oil 2%, paraffin oil 15%, asbestos 2½% and machine oil ½%.

LEON WEISBERG.

75

80

85

90

95

100